

## UNITED STATES PATENT OFFICE.

JOHN M. DONOHUE, OF ROCHESTER, NEW YORK, ASSIGNOR TO EASTMAN KODAK COMPANY, OF ROCHESTER, NEW YORK, A CORPORATION OF NEW YORK.

## CELLULOSE-ETHER COMPOSITION.

No Drawing.

Application filed February 24, 1923. Serial No. 621,087.

*To all whom it may concern:*

Be it known that I, JOHN M. DONOHUE, a citizen of the United States of America, residing at Rochester, in the county of Monroe and State of New York, have invented certain new and useful Improvements in Cellulose-Ether Compositions, of which the following is a full, clear, and exact specification.

10 This invention relates to solvents for making strong solutions of cellulose ether and also relates to the cellulose ether compositions produced by the aid of such solvents. One object of my invention is to provide a 15 solvent which will dissolve such large proportions of cellulose ethers that thick or viscous flowable solutions may be obtained for use in plastic and film making arts. Another object of my invention is to provide 20 a cellulose ether solution which may be manufactured into strong, flexible, transparent films on the machines and by the methods now in use. Other objects will hereinafter appear.

25 In U. S. Patent No. 1,188,376, Lilienfeld, June 20, 1916, there are disclosed a series of alkyl ethers of cellulose. Certain of these are practically insoluble in water, and my invention relates, but is not limited, to the 30 ethers having that property. While cellulose ethers form thin solutions in the formic acid esters of the lower monohydroxy aliphatic alcohols, it has been found that such single solvents by themselves are inadequate 35 to produce the thick flowable compositions or dopes adapted for use in the manufacture of photographic film base by the customary methods or adapted to the other plastic arts.

I have discovered, however, that the formates of the lower monohydroxy aliphatic alcohols have strong latent solvent powers, these powers being brought out by suitable common solvents. By lower monohydroxy aliphatic alcohols I include those having less 45 than 6 carbon atoms. Among the common solvents that may be used are benzol, acetone and the lower monohydroxy aliphatic alcohols. In the formation of film methyl alcohol is preferred.

50 While the ingredients may be mixed in widely varying proportions, it is noted, by way of example, that a particularly useful composition can be prepared by mixing equal parts by weight of the formate and the common solvent. In the preferred form

of my invention, I dissolve 1 part by weight of the cellulose ether, say water-insoluble ethyl cellulose, in from 5 to 7 parts by weight of the solvent mixture, say equal proportions of methyl formate and methyl alcohol. The ingredients by themselves are not sufficiently powerful to make properly flowable dopes of this strength. Of course, the proportion of mixed solvent or the proportion of the volatile ingredients may be increased to adapt the composition to the lacquering art, as will be understood by persons skilled therein.

Other substances which impart additional suppleness, or incombustibility, or other qualities to the film may also be added to the dope, such, for instance, as triphenyl or tricresyl phosphate, monochlornaphthalene, camphor, etc. The ingredients are of the ordinary commercial type and sufficiently purified for the process of film manufacture, so as to give a dope yielding films having the proper relative freedom from color. The viscous-flowable dope above described can be used in connection with the usual film-forming apparatus without the necessity of expensive alterations in the latter.

In the formation of a film by spreading and drying the hereinabove described composition a considerable amount of the formic acid ester remains behind, because of its relatively low volatility, the volatility being less in the esters which have the greater number of carbon atoms in the alkyl radical. The esters impart useful plastifying and other properties to the film, which is normally flexible and transparent. Since the ratio of the weight of alkyl formate to the weight of the cellulose ether can be made much greater by the use of my mixed solvent instead of using the formic acid ester alone as a solvent, it follows that a correspondingly greater proportion of the formate will be present in the finished film than when the cellulose ethers are dissolved in the formic acid esters alone.

Having thus described my invention, what I claim as new and desire to secure by Letters Patent is:

1. A composition of matter comprising cellulose ether and a formic acid ester of a lower monohydroxy aliphatic alcohol and a common solvent which brings out the latent solvent power of the ester.
2. A composition of matter comprising

- cellulose ether and methyl formate homogeneously mixed together in unprecipitated form.
3. A composition of matter comprising 1 part of cellulose ether dissolved in from 5 to 7 parts by weight of a mixture of a formic acid ester in a lower monohydroxy aliphatic alcohol and a common solvent which brings out the latent solvent power of said ester.
- 10 4. A composition of matter comprising cellulose ether dissolved in a mixture of substantially equal parts by weight of a lower monohydroxy aliphatic alcohol and a formic acid ester of a lower monohydroxy aliphatic alcohol.
- 15 5. A composition of matter comprising 2 parts by weight of water-insoluble ethyl
- cellulose, 7 parts of methyl formate and 7 parts of methyl alcohol.
6. As an article of manufacture, a film 20 comprising cellulose ether and methyl formate.
7. As an article of manufacture, a deposited, transparent, flowable film comprising cellulose ether and a formic acid ester 25 of a lower monohydroxy aliphatic alcohol, the proportion of said ester in said film being greater than the maximum proportion depositable in a transparent film from a solution of said cellulose ether in said ester 30 alone.

Signed at Rochester, New York, this 16 day of February, 1923.

JOHN M. DONOHUE.